

# United States Patent Office

2,926,414

Patented Mar. 1, 1960

1

2,926,414

## PRODUCTION OF MECHANICAL EFFECTS ON LIGHT-WEIGHT FABRICS

Ernst Weiss and Fritz Vonaesch, Wattwil, Switzerland, assignors to Heberlein Patent Corporation, New York, N.Y., a corporation of New York.

No Drawing. Application January 18, 1955  
Serial No. 482,655

Claims priority, application Austria April 15, 1954

3 Claims. (Cl. 26—69)

This invention relates to a process for producing mechanical pattern or all-over effects, such as embossing and plain calender effects on fabrics, especially light-weight fabrics.

The expression "light-weight fabrics" as herein used is intended to refer to cotton fabrics having a count in the order of 45 to 150 threads per inch and English yarn numbers of 50 to 200 in the warp and filling. Such fabrics are exemplified by, but not restricted to, cotton muslins, cotton voiles, percale and cotton Geisha fabrics as referred to herein below.

We have found, in accordance with our invention, that the application of heat-setting resins to such light-weight fabrics with subsequent application of goffering, friction calendering or similar relatively rough mechanical processing causes severe strains in such light-weight fabrics and they frequently break or tear during the process to cause a large proportion of "seconds." This is not only true in all-over treated fabrics, but it is also especially true in cases, where the mechanical effects are to be applied in the form of pattern effects, resulting in fabrics which will be only partly covered with a durable lustrous finish or an embossed effect.

The principal object of this invention, accordingly, is to provide a simple efficient process for such treatment of light-weight fabrics, which shall substantially overcome the difficulty mentioned and produce a series of products having the effects mentioned.

The invention accordingly consists of the novel products as well as the novel processes and steps of processes according to which such products are manufactured, the specific embodiments of which are described hereinafter by way of example and in accordance with which we now prefer to practice the invention.

In accordance with our invention we use a light weight fabric having a count in the order of 45 to 150 threads per inch and English yarn numbers of 50 to 200 in the warp and filling, that has previously been shrunk. To this fabric a resin precondensate is applied, whereupon it is mechanically treated as by calendering to give an embossed, Schreiner, moire or plain calendering effect, for example. The fabric is then heated to set the resin. The product so prepared is a shrunk light-weight cotton fabric having a mechanical effect thereon of the kind mentioned above, either as an over-all effect or as a patterned effect which is permanently fixed by means of a thermosetting resin. The preshrinking of the light weight fabric is performed with caustic soda solution of about 22-30° Bé. or caustic potash solution of about 24-30° Bé. Such shrinkage may be effected at any time in the process prior to the application of the resin precondensate. That is, it may be carried out on the grey goods or may be carried out after kier-boiling or after the bleaching of such grey goods.

The light-weight fabrics which may be employed include cotton muslin, cotton voile, percale and cotton Geisha cloth. For the production of local mechanical

2

effects, fabrics pre-dyed in lighter shades and/or color printed fabrics can be provided in conformity to the designated pattern with a resin compound containing color pigment if desired. The usual color printing can be applied side by side of the resin printing. If darker shades are desired next to light-colored mechanical effects, the fabric may be subsequently dyed for this purpose.

The resin precondensates are heat-setting synthetic resins and include the following: condensates of formaldehyde with urea, thiourea, ethylene urea and homologues of same, acetylene diurea and derivatives thereof, dicyandiamide, melamine, and condensates of formaldehyde and phenol and phenol derivatives, as well as suitable mixtures of these resin precondensates. Furthermore ketone-aldehyde and dimethylolurone precondensates are suitable. All these synthetic resin precondensates are applied on the fabric in the form of an aqueous solution in the presence of the usual acid or alkaline catalysts. Also suitable soluble dye-stuffs, white or colored pigments, or compositions forming same, as well as metal powder can be added to the solution together with the dye-stuffs as desired.

With respect to the production of local mechanical effects, that is pattern effects such as goffered or the like, we produce such goffered or similar effect all over the fabric and then set the locally applied resin and then treat the fabric with a dilute swelling agent solution such as dilute caustic soda solution for the purpose of completely eliminating the goffered or like effect from the fabric background.

In case undulation of the local mechanical effect is desired, the fabric can be thereafter treated with an alkali lye of mercerizing strength. On the other hand, if transparentizing or parchmentizing of the fabric background is desired, this may be accomplished by treatment with sulphuric acid of suitable strength.

The following are examples of the process in accordance with our invention as we now prefer to practice it. These examples are purely illustrative and the invention is not to be considered as restricted thereto except as indicated in the appended claims.

### Example 1

45 A conventionally kier-boiled and bleached cotton muslin fabric with 105 ends and 90 picks per inch and the English yarn numbers 100 and 120 in the warp and filling or weft is impregnated on a padder with caustic soda solution of 22° Bé., kept in this condition several minutes, then de-leyed hot and cold and dried loose. Hereupon, the fabric is impregnated with the following composition:

|                                                                                                                               | Gr.  |
|-------------------------------------------------------------------------------------------------------------------------------|------|
| 55 Cassurit. MKF (polymethylol melamine precondensate of Cassella Farbwerke Mainkur, Germany) -----                           | 90   |
| Water -----                                                                                                                   | 200  |
| 60 Ahcovel G (fatty carbamide of Arnold Hoffman Co., Providence, R.I., U.S.A., see U.S.A. Patents 2,304,113, 2,304,369) ----- | 10   |
| Gum tragacanth—1 gum:10 water-----                                                                                            | 100  |
| 65 Catalyster C (triethanolamine glycolate of Cassella Farbwerke Mainkur, Germany) -----                                      | 9    |
| Water -----                                                                                                                   | 491  |
|                                                                                                                               | 1000 |

70 predried at 40° C., embossed at 200° C., cured at 140° C. for 5 minutes, washed out cold and warm and dried on a tenter frame.

## Example 2

A cotton muslin fabric with 90 ends and 82.5 picks per inch and the English yarn numbers 80 and 120 in the warp and the filling or weft is de-sized and kier boiled according to the usual methods. Thereupon it is impregnated with caustic soda solution of 30° Bé., kept in this condition for five minutes, de-lyed hot and cold, beached, rinsed, centrifuged and dried under low tension. Hereupon, in conformity with the designated pattern, the fabric is printed with the following composition:

|                                                                                                 |      |    |     |
|-------------------------------------------------------------------------------------------------|------|----|-----|
| Lyofix CH (hexamethyol melamine precondensate of Ciba A.G., Basel, Switzerland)                 | 100  | 15 | Gr. |
| Tylose TWA 50:1000 (methyl cellulose of Kalle & Co. A.G., Wiesbaden-Bieberich, Germany)         | 500  |    |     |
| Ahcovel G (see Example 1)                                                                       | 40   |    |     |
| Polyvinyl alcohol 12%                                                                           | 50   |    |     |
| Indanthren gold yellow RK suprafix double paste (Schultz index, supplementary volume No. 1286c) | 100  |    |     |
| Ammonium chloride/water 1:1                                                                     | 10   |    |     |
| Water                                                                                           | 200  |    |     |
|                                                                                                 | 1000 |    |     |

Following this the fabric is pre-dried at 50° C., embossed on a goffering calender at 200° C., cured for 4 minutes at 140° C., washed and dried. Thereafter, in order to remove the embossing completely from the unprinted part of the fabric, it is treated for some time in a bath containing caustic soda solution of 20° Bé. and 10 gr. Invadine ME<sup>1</sup> per liter, de-lyed hot and cold, rinsed and dried on a tenter frame.

## Example 3

A cotton percale fabric, the count of which is 105/98 ends and picks per inch, English yarn numbers 50/60, is kier boiled and bleached in the usual manner and then impregnated with caustic potash solution of 25° Bé. and kept in this condition as in the foregoing examples, then de-lyed and dried under light tension. Hereupon, in conformity with the designated pattern, the fabric is printed with the following composition:

|                                                                                            |      |     |
|--------------------------------------------------------------------------------------------|------|-----|
| Bekamine P 468 (ketone aldehyde precondensate of Reichhold Chemical Inc., Detroit, U.S.A.) | 175  | Gr. |
| Water                                                                                      | 100  |     |
| Alkagum 60:1000 (carob bean meal thickener)                                                | 500  |     |
| Indanthrene blue GCD (Schultz index No. 1234)                                              | 100  |     |
| Soda calc.                                                                                 | 14   |     |
| Water                                                                                      | 111  |     |
|                                                                                            | 1000 |     |

Following this the fabric is pre-dried at 45° C., embossed at 240° C., cured for 3 minutes at 150° C., washed and dried. Thereafter, in order to remove the embossing completely from the background, it is impregnated with caustic potash solution of 20° Bé. on a pad, kept in that condition for some time, de-lyed hot and cold, rinsed and dried on a tenter frame.

## Example 4

A light-weight cotton fabric known under the name of "Geisha" (ends and picks per inch 105/90, English yarn numbers 80/95) is de-sized and kier-boiled according to the usual methods. Thereafter, it is impregnated with caustic potash solution of 30° Bé., kept in this condition for several minutes, de-lyed hot and cold, bleached, rinsed, centrifuged and dried loose. Here-

<sup>1</sup> Mercerizing auxiliary agent containing phenolic compounds of Ciba A.G., Basel, Switzerland.

upon, in conformity with the designated pattern, the fabric is printed with the following composition:

|    |                                                                                                                                  |      |     |
|----|----------------------------------------------------------------------------------------------------------------------------------|------|-----|
| 5  | Cassurit MKF (see Example 1)                                                                                                     | 80   | Gr. |
|    | Water                                                                                                                            | 400  |     |
|    | Traganth 1:10                                                                                                                    | 75   |     |
|    | Catalyzer C (see Example 1)                                                                                                      | 8    |     |
|    | Water                                                                                                                            | 436  |     |
| 10 | Hostapal C (condensation product of an alkylphenol with ethylene oxide of Hoechst Dye Works, Frankfurt am Main Hoechst, Germany) | 1    |     |
|    |                                                                                                                                  | 1000 |     |

Following this the fabric is pre-dried at 40° C., embossed at 200° C. on a Riffle or shallow embossing calender and aftertreated as described in Example 1.

## Example 5

20 A cotton muslin fabric with 90 ends and 71 picks per inch and the English yarn numbers 80/120 in the warp and the filling or weft is singed, impregnated in a dry, raw state with caustic soda solution of 25° Bé. to which 10 gr. Invadine ME (see Example 2) was added per liter and kept in the impregnated state for 8 minutes. Thereupon the fabric is de-lyed hot and cold, kier-boiled and bleached according to the usual methods, rinsed, centrifuged and dried under light tension. Hereupon, in conformity with the designated pattern, the fabric is printed with the following composition:

|    |                                                         |      |     |
|----|---------------------------------------------------------|------|-----|
| 30 | Lyofix CH (see Example 2)                               | 120  | Gr. |
|    | Ahcovel G (see Example 1)                               | 40   |     |
|    | Tylose TWA 50:1000 (see Example 2)                      | 500  |     |
| 35 | Indanthrene red RK, fine paste (Schultz index No. 1258) | 100  |     |
|    | Ammonium thiocyanate/water 1:1                          | 10   |     |
|    | Water                                                   | 230  |     |
|    |                                                         | 1000 |     |

Following this the fabric is pre-dried at 40° C., led twice through a friction calender at 180° C., cured for 4 minutes at 140° C., washed warm and cold and finished in the usual manner.

## Example 6

45 A cotton muslin fabric with 105 ends and 90 picks per inch and the English yarn numbers 80/100 in the warp and the filling or weft, kier-boiled and bleached in the usual manner, is impregnated with a caustic soda solution of 22° Bé., kept in this condition for several minutes, de-lyed and dried under light tension. Hereupon the composition described in Example 2 is printed on the fabric in conformity to the designated pattern. Then the fabric is pre-dried at 40° C., embossed on a goffering calender at 220° C., cured for 4 minutes at 140° C., washed and dried. The dry fabric is impregnated with caustic soda solution of 38° C., then kept in a tensionless state for three minutes, de-lyed hot, thereafter rinsed with cold water and dried under slight tension. One obtains embossed and, depending on the pattern, more or less undulated print sections on a shrunken background.

65 70 A fabric, treated according to Example 5, after the resin has been cured and the fabric has been washed and framed, is impregnated with caustic soda solution of 38° Bé., kept in a tensionless condition for 3 minutes, de-lyed hot, thereafter rinsed with cold water, dried in a loop dryer and steamed with little tension on a tenter frame. One obtains lustrous, more or less undulated print sections, depending on the pattern, on a shrunken background.

What we claim is:

1. A process for producing mechanical calendering effects upon a light-weight cotton fabric, which comprises shrinking with an aqueous alkali solution of cotton shrinking strength a cotton fabric which is subject to damage under rough mechanical processing when having a thermosetting resin precondensate thereon, said fabric having a count of 45 to 150 threads per inch and English yarn numbers of 50 to 200 in the warp and filling, applying a thermosetting resin precondensate to the shrunk fabric, mechanically treating the fabric with a hot calender to impart a desired mechanical effect to the fabric without substantial injury thereto, and then heating the so-treated fabric to cure the resin precondensate and set the effect in the fabric.

2. A process as set forth in claim 1 wherein the aqueous alkali solution of cotton shrinking strength is selected from the group consisting of about 22 to 30° Bé. caustic soda and about 24 to 30° Bé. caustic potash.

3. A shrunk light-weight cotton textile fabric of a count of 45 to 150 threads per inch and English yarn numbers of 50 to 200 in the warp and filling having a

permanently fixed mechanical calendering effect thereon produced by the process of claim 1.

References Cited in the file of this patent

UNITED STATES PATENTS

|    |           |                  |               |
|----|-----------|------------------|---------------|
| 5  | 1,925,914 | Zanker           | Sept. 5, 1933 |
|    | 2,119,150 | Bowen et al.     | May 31, 1938  |
|    | 2,121,005 | Bener            | June 21, 1938 |
| 10 | 2,123,153 | Rivat            | July 5, 1938  |
|    | 2,161,223 | Bener            | June 6, 1939  |
|    | 2,353,225 | Dreyfus          | July 11, 1944 |
|    | 2,370,946 | Finlayson et al. | Mar. 6, 1945  |
|    | 2,517,529 | Stanley          | Aug. 1, 1950  |
| 15 | 2,590,402 | Hall et al.      | Mar. 25, 1952 |
|    | 2,699,374 | Bener            | Jan. 11, 1955 |
|    | 2,733,998 | Russell          | Feb. 7, 1956  |
|    | 2,743,190 | Vonaesch         | Apr. 24, 1956 |

FOREIGN PATENTS

|    |         |               |                |
|----|---------|---------------|----------------|
| 20 | 592,649 | Great Britain | Sept. 24, 1947 |
|    | 607,582 | Great Britain | Sept. 1, 1948  |
|    | 695,703 | Great Britain | Aug. 19, 1953  |